

# UNITED STATES PATENT OFFICE

ENGBERT HARMEN REERINK AND JOHANNES GIJSBERTUS WILHELM MULDER, OF EINDHOVEN, NETHERLANDS, ASSIGNORS TO RADIO CORPORATION OF AMERICA, A CORPORATION OF DELAWARE

## WEHNELT-CATHODE

No Drawing. Application filed April 4, 1929, Serial No. 352,597, and in the Netherlands April 13, 1928.

The invention concerns cathodes, more particularly, Wehnelt-cathodes, and the process of manufacturing the same, and has for its object the provision of a cathode having long life. As is known, a Wehnelt-cathode contains metallic compounds, such as oxides, which when heated emit electrons.

In our invention, the Wehnelt-cathode contains, in addition to the active emitting compound consisting, for example, of barium or a barium compound, a beryllium compound, preferably beryllium oxide. This has been found to increase the life of the cathode. Particularly good results are obtained by adding also a zirconium compound, preferably zirconium oxide. A cathode which, in addition to the active emitting compound, contains both a beryllium and a zirconium compound, has proved to possess better emitting and lasting properties than a cathode which contains only a beryllium compound or only a zirconium compound.

Such a Wehnelt-cathode can be manufactured by coating a core with a suspension of barium carbonate, beryllium carbonate, zirconium oxide, and if desired, an agglutinant, e. g. gum arabic, and by subsequently heating the body, preferably in a vacuum, and preferably to a temperature of about 1000° C. The core may, for example, be a nickel wire, or a tungsten wire having helically wound on it a nickel wire.

I claim:

35 A process of manufacturing a Wehnelt-cathode, in which the core is coated with a suspension of barium carbonate, beryllium carbonate, zirconium oxide and an agglutinant, and is subsequently heated in a vacuum.

40 ENGBERT HARMEN REERINK.  
JOHANNES GIJSBERTUS WILHELM MULDER.